

June 23, 1931.

F. J. HOXIE ET AL.

1,811,395

## METHOD FOR INCREASING THE TENSILE STRENGTH OF YARNS

Filed March 19, 1926

Fig. 2



Fig. 1.



*INVENTORS:*  
*Frederick J. Hoxie*  
*Ashton M. Tenney.*

Ashton M. Tern  
BY  
Harold J. Penney, ATTORNEY

## UNITED STATES PATENT OFFICE

FREDERICK J. HOXIE, OF PHENIX, RHODE ISLAND, AND ASHTON M. TENNEY, OF NEW ROCHELLE, NEW YORK, ASSIGNEES, BY DIRECT AND MESNE ASSIGNMENTS, OF ONE-HALF TO WELLINGTON, SEARS & COMPANY, OF NEW YORK, N. Y., A FIRM CONSISTING OF HARRY L. BAILEY, NORMAN S. HOPE, JOHN H. BENNETT, AND CHARLES O. RICHARDSON, AND ONE-HALF TO WARWICK MILLS, OF WEST WARWICK, RHODE ISLAND, A CORPORATION OF RHODE ISLAND

## METHOD FOR INCREASING THE TENSILE STRENGTH OF YARNS

Application filed March 19, 1926. Serial No. 95,978.

Our present invention relates to an improvement in methods for increasing the tensile strength of yarns and textile threads of a similar nature, such as will be hereinafter disclosed.

This improvement is also directed to the provision of apparatus whereby the herein-after to be outlined methods of treatment are carried out, such illustration being in a more or less diagrammatic manner.

One of the main advantages of our invention relates to the manner in which yarns may be treated (in the skein) for strengthening the same so that they may be readily utilized thereafter in looms for weaving, and whereby the tensile strength of such yarns may be increased so as to prevent breakage during the weaving process.

Another advantage of our invention lies in the fact that after the treatment has been carried out on yarns and woven into fabrics, the results of the treatment may be removed by the mere process of washing, thereby leaving the fabric in a condition that it originally would have been had the yarn been untreated, with the exception that the yarn has been woven into a fabric unbroken and unstretched, and therefore without any defects in this respect.

Another advantage of our invention resides in the manner in which the yarn may be treated in bulk, or in large masses, so that the cost thereof is greatly reduced.

These and other capabilities will be ascertained as the description herein proceeds and it is understood that modifications may be made in the process and apparatus herein outlined without violating the scope of the invention as herein disclosed.

While our invention is directed to certain classes of yarns, which are normally very weak, it is more especially directed to the treatment of artificial silk known in the trade, at present as "rayon", which, as is well known, lacks tensile strength in the yarn, and this failing very often creates difficulties in the weaving thereof owing to the breakage or stretching of the yarn, which has not been, up till now, controlled.

For the purpose of strengthening the yarn

without affecting its pliability, prior to the weaving thereof into desired fabrics, in order to do away with breakage and to prevent the stretching of the yarn during weaving, thereby creating what is known as "shiners" in the completed fabric, we have ascertained that rayon, being insoluble and non-absorbent in its nature, may be treated in the skein with a coating of water-soluble quick-drying size or adhesive dressing materials, which are sufficiently flexible when dried to permit of weaving. One satisfactory material is gelatine, which, after the yarn has been coated, may be sufficiently dried and manipulated in such a manner as to permit the mass of threads within the skein to be fluffed and kept individually separated, thereby leaving the skeins in condition to be wound upon bobbins, the threads of said skeins being separate, one from the other, notwithstanding the fact that they were treated and dried in a skein mass.

A further step during the process is the provision of means whereby after the gelatinous coating has been placed upon the yarn it is possible to evenly distribute the coating upon the thread to any predetermined thickness. This is the deciding factor of what the added tensile strength of the thread may be and also its residual flexibility, sufficient for weaving purposes.

Our invention also contemplates the further provision of a step wherein the gelatine-treated yarn, after such treatment, including the control of the thickness of the coating thereon, may be rapidly dried by artificial heating means whereby the moisture content of the hygroscopic coating may be rapidly extracted therefrom and during such extraction, the reaction thereof will be conducive to the permanent separation of the threads forming the skein, as such, and prevent their adhering, thereby to form a mass.

In the accompanying drawings:

Fig. 1 is a sectional view of a circular form of machine, taken on the section lines 1—1, Fig. 2;

Fig. 2 is a plan view of the apparatus with the cover and skeins removed.

By referring to Fig. 1, there is shown in

section a structural apparatus in which our process is carried out and in general comprises a non-rotatable frame casing, generally denoted by 1, having side walls 2 and a base flange 3 which in turn is suitably and immovably affixed to a base plate B. At the upper end of the frame 1 is located a sheet metal pan or housing, generally denoted by 4, which has an annular upstanding edge 5 and a sloped bottom 6 which is provided with an upturned inner flange 7, the function of which will be later described.

10 The upper pan 4 is provided with a fairly tight closing cover 8, which is removable therefrom upon occasion.

15 At the center of the housing there is provided a bearing 9 in which is mounted a revolvable spindle 10, at the bottom end of which is suitably affixed thereto, for driving, 20 a bevel gear 11 which in turn meshes with a bevel pinion 12 which is driven at suitable speeds by an electric motor M which is suitably mounted to the base 1 as shown.

25 The upper end of the spindle 10 carries on its upper flange 13, a revolvable pan or centrifuge 14, the sides of which are preferably sloping or flared outwardly as shown.

30 At predetermined intervals as at 15, Figs. 1 and 2, there are mounted to the bottom of the pan, any desired number of fixed skein pegs 15 and in radial alinement therewith and near the center thereof, there are mounted an equal number of adjustable skein pegs 16, these being set in gibways 17, so that 35 the pegs 16 may be adjustably set to suit the length of the skeins of yarn 18, which are mounted on said pegs 15 and 16, as shown in Fig. 1. In actual practice either one or both of these paired pegs may be adjustable for 40 the purpose of taking up slack in the skein and holding the skeins rigidly in desired radial position in order to meet the subsequent treatments and the later centrifugal action given, as will be later described.

45 At the lower end, and preferably within the base 1, are located two reservoirs G and O, one of which G, carries within it a liquid solution of gelatine or any equivalent coating material that may be found suitable for the 50 purpose. The opposite reservoir O is filled with a heatable material, such as mineral oil, of suitably high boiling point.

Under the oil reservoir O means are provided, such as a multiple gas burner H where- 55 by the oil in the reservoir may be suitably heated, fuel for this purpose being supplied through the duct D, from any suitable source of supply.

60 Intermediate of the two reservoirs, are located two small electric motors E which in turn drive two small fluid pumps P by means of belts L or any other suitable form of drive connection.

65 All of the electric motors, including M, may be controlled by independent switch

means, not shown, which may be located outside of the apparatus whereby each of them, in their predetermined sequence, may be caused to operate, by manual control to carry out the sequential treatments of the skeins. 70

The pumps P have ducts S, which run to the lower portion of the said pumps from their respective reservoirs, and form inlets thereto, and at the pump outlet ends are connected to internal ducts T, the outlets of 75 which end within the interior of the centrifuge 14 as at U, Fig. 1. These upstanding, fixed ducts T—U are supported within the stationary spindle V which runs through the center of the spindle 10, and which is rigidly 80 mounted upon the base B.

On opposite sides of the housing 1 are provided drain pipes W suitably mounted to receive the drainage of their respective fluids, as will be later described, whereby the said 85 fluids may be conducted back to their respective reservoirs and these ducts are controlled by hand valves or other suitable means.

In order to carry out our herein process, a plurality of skeins 18 are mounted upon the 90 skein pegs 15, 16 which pegs are adjusted to hold the skeins rigidly in a, preferably, radial position to the axis of the centrifuge.

The cover 8 is thereupon closed and the switch for starting the motor E, for pumping gelatine, is then closed. This causes the centrifuge 14 to become filled with liquid gelatine from the reservoir G. The gelatine pump is stopped when a predetermined amount of gelatine has been provided in the 100 centrifuge 14. The motor M is started, and this causes the centrifuge 14 to rotate at high speed and discharge all of the excess gelatine to be thrown into the drain pan 4, the hand valve X controlling the drainage of the gelatine back to the reservoir G is opened and the excess gelatine is thereafter caused to flow back into said reservoir for reuse. 105

The centrifuge 14 may be revolved until all excess gelatine has been removed from the skeins leaving them coated to any desired degree with a thin external coating upon the threads thereof, thereafter the gelatine drain pipe is closed, the motor M is stopped, and the motor E controlling the heated mineral oil from the reservoir O is then caused to pump the heated oil, into the centrifuge, until the centrifuge 14 is filled and covers the skeins. 110

The flow of hot oil is then stopped, the motor M started and the centrifuge again revolved at high speed thereby discharging the hot oil into the upper pan 4 where it is returned to its reservoir O, by means of the hand valve X and the spinning of the centrifuge 14 is continued until the required amount of excess oil is removed from the threads. 120

125 After the foregoing described operation, the motor M is stopped, the oil hand valve X 130

is closed, the cover 8 and the skeins 18 are removed from the apparatus and the filling and treating with another lot of skeins is again repeated.

- 5 In the treatment of the skeins as above described, and owing to the insoluble condition of the rayon, it is obvious that the introduction of liquid gelatine upon the skeins causes the same to become thoroughly coated and 70  
10 whirling the skeins thereafter causes the same to be deprived of all excess gelatine leaving the skeins with a desired coating of gelatine thereon, depending on the amount of centrifugal action they receive, this being under 75  
15 control.

Thereafter, upon the introduction of the hot oil, a peculiar phenomenon takes place, that is to say, that when the oil which may be heated to, not in excess of 250 degrees F. is 80  
20 introduced upon the skeins, the heat thereof causes an immediate change of the moisture content of the skeins into steam and this action, while substantially instantaneous, causes the threads of the skein to become violently separated and fluffed away from one another at or about which point the centrifuge is started and the excess hot oil is driven off and strands of the skein kept separated by the centrifugal action of the rotating 85  
25 centrifuge.

- 30 The gelatine coating upon the strands has in the meantime become thoroughly dried due to the heated oil and the skeins are thereafter removed in a flexible, pliable, condition 90  
35 having a dried coat of gelatine thereon which increases the tensile strength of the said threads without appreciably changing the texture or workable condition and with a thin coating of oil thereon which rather favors 95  
40 the later operation of weaving into fabrics.

After the rayon, so strengthened, has been woven into a fabric, the fabric may then be treated in a hot water bath and all of the oil and gelatine thereafter removed, leaving the 100  
45 fabric in a clean condition and without the customary defects which have heretofore been met with when rayon has been woven without treatment, as set forth above. Of course the coated strands can be sold in skein 105  
50 form to weavers.

We do not desire to be limited to the treatment of yarns in the skein, nor to treating the yarns with gelatine only, as we have ascertained that there are other size or adhesive 110  
55 dressing materials such as gums or their equivalents, albumens, starch, dextrin, or glucose that may be used which answer the purpose fully. It is to be further understood that we are not limited to mineral oil as the 115  
60 heating fluid. Any oil that will not harm the artificial silk or coating is suitable.

Hot oil may be arranged to flow continuously into the centrifuge while the centrifuge is slowly revolving thereby making the action substantially continuous and without de- 120  
65

parting from the scope of the invention herein outlined.

Other forms of apparatus may be also used, to carry out the sequential steps herein outlined, other than the forms herein illustrated. 70

Having thus described our invention, what we claim is:

1. The process of coating yarns in the skein for increasing the tensile strength thereof which consists in immersing the yarn in an aqueous solution of gelatine, subjecting said yarn to whirling, then immersing said yarn in a heated oil the temperature of which is above the evaporating point of the water in said gelatine solution, to vaporize said water, then whirling the yarn to remove the heated oil. 80

2. The process of treating yarns for increasing the tensile strength thereof which consists in immersing the yarn in a solution of gelatine, to coat the same, then treating the said yarn by whirling to remove the excess gelatine, then immersing said yarn in a heated oil the temperature of which is above the evaporating point of the solvent of said gelatine, to evaporate said solvent, then whirling the yarn to remove the heated oil. 85

3. The process of increasing the tensile strength of rayon which consists in treating skeins of rayon with a gelatine solution, drying said gelatine by a heated oil to a point which will remove, by evaporation, the solvent of said gelatine, leaving the gelatine in a dry condition and as a coating upon said rayon, subjecting the rayon skein to a whirling action during such treatment thereby to remove the excess gelatine and oil and thereby to fluff the rayon skein so that the individual threads of rayon are dried and kept separate one from another in the skein mass. 90

4. The process of treating rayon threads in a skein to increase the tensile strength thereof which consists in, first, causing an immersion of the said threads in liquid water soluble gelatine, whirling the same to remove the excess of said gelatine, then causing an immersion of the rayon skein in a bath of heated oil to cause rapid evaporation of the solvent of said gelatine, to dry the same during which action the solvent is violently dissipated from the said gelatine and through the vapor caused thereby, to cause the individual threads of the skein, as treated, to become separated one from the other and to then whirl the said skein thereby driving off all the excess of the oil and completing the separation of the threads in the skein, through such centrifugal action. 100  
110

5. The process of treating rayon threads to increase the tensile strength thereof which consists in, first, causing an immersion of the said threads in a gelatine solution, whirling the same to remove the excess of said gelatine and to coat the threads, then causing an immersion of the threads in a bath of heated 115  
120  
125  
130

oil to cause rapid evaporation of the solvent of said gelatine during which action the solvent is violently dissipated from the said gelatine and through the vapor caused thereby causes the threads to become dried, to prevent sticking to one another and then whirling the said thread thereby driving off all the excess of the oil and completing the drying of the threads through such whirling action.

10 6. A process for increasing the tensile strength of yarns which consists in treating a yarn skein with a water-soluble adhesive sizing adapted to strengthen the yarn, and simultaneously subjecting said skein to centrifugal action and heated numeral oil whereby each yarn thread is separately dried.

15 7. A process for increasing the tensile strength of yarns which consists in coating a yarn skein with a water-soluble, rapidly drying adhesive sizing, and simultaneously subjecting said skein to heated mineral oil and rotation whereby each yarn thread is individually dried.

20 8. A process of increasing the tensile strength of threads, which includes the steps of treating the thread by immersion in a water soluble adhesive sizing adapted to strengthen said thread for weaving of said thread into a fabric, then subjecting the 25 thread to whirling action to remove the excess sizing therefrom leaving a strengthening coating on said thread, immersing said coated thread in heated oil at a temperature above the evaporating point of the sizing solvent, and then subjecting the thread to further whirling action whereby excess oil is removed and said thread is left with said strengthening coating thereby rendering it suitable for weaving into fabric.

30 40 9. A process of increasing the tensile strength of threads which includes the steps of treating the thread by immersion in a gelatine solution, subjecting the thread to a whirling action thereby leaving a gelatine 35 coating on said thread, adapted to strengthen said thread when said thread is being woven into fabric, immersing said gelatine coated thread in heated oil to remove the water in said gelatine, and then subjecting the 45 thread to whirling action to remove excess oil and dry said coated thread.

50 10. A process for strengthening rayon threads of low tensile strength which consists in subjecting the threads to a gelatine 55 solution, and then simultaneously subjecting said threads to centrifugal action and heated mineral oil whereby the coating on each thread individually is dried.

60 11. As a new product, applicable for the weaving of fabric, a skein of yarn, the threads of which are normally of low tensile strength, coated with gelatine on each of said threads whereby the tensile strength of said threads 65 is increased and a film of oil on said gela-

70 tine whereby weaving of said threads is facilitated.

75 12. A process for increasing the tensile strength of yarns, which consists in coating a yarn skein with an aqueous solution of a suitable adhesive dressing adapted to strengthen the yarn, then removing the excess of said dressing solution and then simultaneously drying said skein by means of a non-aqueous fluid having a sufficiently high temperature and centrifugally treating said skein to separate the yarn threads in the skein from one another.

80 13. A process for strengthening rayon threads of low tensile strength, which consists in coating said threads with gelatine by immersing said threads in an aqueous gelatine solution and then evaporating the water of the solution by means of a non-aqueous fluid having a suitable temperature and, while said evaporating action is progressing, subjecting the threads to a centrifugal action.

85 Signed at New York, in the county of New York and State of New York, this 18th day of March, A. D. 1926.

90 FREDERICK J. HOXIE.  
ASHTON M. TENNEY.

95

100

105

110

115

120

125

130